

## UNITED STATES PATENT OFFICE

2,327,155

## PROCESS FOR TREATING WAX

Ralph C. Pollock, Long Beach, Calif., assignor to  
Union Oil Company of California, Los Angeles,  
Calif., a corporation of California

No Drawing. Application March 6, 1939,  
Serial No. 260,114

5 Claims. (Cl. 196—78)

The present invention relates to a process for producing lubricating oil. The invention also relates to a process for producing wax crystallization modifiers or wax separation aids and also pour point depressants for lubricating oils. The invention relates particularly to a process for producing lubricating oils of high viscosity index or low viscosity gravity constant from paraffin wax, such as scale wax and slack wax, in particular oxidized wax.

I have discovered that valuable lubricating oil of extremely high viscosity index may be produced from paraffin wax by subjecting the paraffin wax to oxidation followed by thermal decomposition or cracking and separating the lubricating oil contained in the cracked oxidized wax.

In general, the oxidized paraffin wax from which the valuable lubricating oil may be produced by cracking is prepared by subjecting an unoxidized paraffin wax to the action of an oxygen-containing gas such as air, oxygen or ozone, preferably at an elevated temperature. The condition and degree of oxidation will vary with the type and oil content of the wax, with temperature of oxidation, with the air rate and whether or not a catalyst is employed. Generally, I prefer to oxidize the paraffin wax for a relatively long period of time, for example 75 hours to 400 hours, while maintaining the charge at a relatively low temperature of the order of 200° F. to 350° F.

If desired, the oxidation may be carried out in the presence of a catalyst. Catalysts which may be employed for this purpose are metal chlorides, such as chlorides of iron, zinc, tin, aluminum; metal soaps, such as naphthenates (oleates, stearates, ricinoleates, palmitates) of sodium, copper, magnesium, manganese, aluminum, cobalt, iron and nickel. I have obtained good results by using above 0.5% by weight of nickel naphthenate. The oxidation may also be carried out with hydrogen peroxide while maintaining the charge at an elevated temperature. If desired, air may be simultaneously introduced into the heated charge of paraffin wax while adding hydrogen peroxide to the charge or the air may be passed through a separate vessel containing hydrogen peroxide and the activated air or oxygen thence passed into the heated charge.

The degree of oxidation may be determined approximately by measuring the acid and saponification numbers of the oxidized charge. When oxidizing scale wax, for example, it is preferable to stop the oxidation reaction when the charge shows a saponification number of approximately 140 to 160 and an acid number of approximately

40 to 50. The cracking of the oxidized paraffin wax is preferably carried out under such controlled conditions as to prevent the production of coke-like materials in the residue resulting from the cracking distillation. Preferably, the cracking reaction is carried out at low temperature at not appreciably above 700° F. If desired, the cracking reaction may be carried out in the presence of a catalyst such as aluminum chloride, aluminum oxide, zinc chloride, stannic chloride, etc.

During the cracking of the oxidized paraffin wax, water is formed due to the splitting off of hydrogen and oxygen molecules from the oxygenated paraffin wax. Light oils resembling gasoline, gas oil and kerosene are also produced. The water and light oils thus formed are preferably removed from the cracked paraffin wax by distillation which may be carried out during or subsequent to the cracking reaction. The cracking also results in the splitting off of light volatile acids.

The bottoms thus produced from the cracking reaction contain the valuable lubricating oils of high viscosity index and also unconverted wax. The high viscosity index lubricating oil may be recovered from these cracked bottoms by dissolving them in a diluent and chilling the mixture to a sufficiently low temperature to crystallize the unconverted wax content and subsequently separating the precipitate of wax and other materials hereinafter discussed as wax modifiers which are insoluble in the solution at the low temperature by known methods of filtration, cold settling or centrifuging. As diluents for this purpose, I may employ any of the known diluents in which the oil is soluble at the low temperature to which the solution is chilled but in which wax is insoluble. I may employ liquefied normally gaseous hydrocarbons such as ethane, ethylene, propane, propylene, butane, butylene or mixtures thereof, like liquid hydrocarbons such as pentane, hexane, heptane, octane, nonane or hydrocarbon fractions such as naphtha, gasoline, kerosene or gas-oil or I may employ such diluents as acetone, methyl ethyl ketone, diethyl ketone, methyl propyl ketone, ethyl propyl ketone, mixtures of these ketones with benzene, ethyl alcohol, propyl alcohol, butyl alcohol, cyclohexanone, normally gaseous and normally liquid ethers, methyl chlorides, dichloroethylene or trichloroethylene or mixtures of these materials with the aforementioned hydrocarbons.

The use of liquefied normally gaseous hydrocarbons, such as liquid propane, is preferred

since in addition to having the property of retaining less wax in solution at low temperatures, it may be employed to produce the necessary degree of refrigeration to precipitate the wax from the solution. This is accomplished by reducing the pressure of the mixture and allowing a portion of the liquefied normally gaseous material from the diluent-oxidized wax mixture to vaporize.

The diluted oil subsequent to its separation from the precipitate by filtration, cold settling or centrifuging is, of course, heated to distill off the diluent. If desired, the thus recovered oil may be separately purified by acid treatment followed by alkali and/or clay treatment or it may be blended with other dewaxed lubricating oils and the blend of oils then purified by acid, alkali or clay treatments. Due to the extremely high viscosity index of the lubricating oil recovered from the oxidized wax, this oil may be used as a blending material for oils of relatively low viscosity index in order to raise the viscosity index of the latter. If desired, a further improvement in viscosity index of the extracted oil may be obtained by subjecting the oil to extraction with selective solvents such as phenol, furfural and the like.

I have further discovered that the cracked bottoms of the oxidized paraffin wax contain, in addition to the valuable lubricating oil heretofore mentioned certain materials which are quite active in conditioning waxy oils to be dewaxed so that the wax may be more readily separated from the oil. When small amounts of these materials, for example, 0.5 to 2.0%, are added to lubricating oils to be dewaxed by chilling and filtration, an improvement is obtained with respect to the yield of dewaxed oil, filter rate or rate of wax separation and melting point of the separated wax.

The active wax modifier may be recovered from the cracked oxidized bottoms by mixing the cracked bottoms with a solvent capable of dissolving oil and wax contained in the cracked bottoms but which will not dissolve appreciable quantities of the wax separation aid. For this purpose, I may employ any of the solvents heretofore mentioned, preferably the liquefied normally gaseous hydrocarbons, specifically liquid propane. When, for example, 10 volumes of liquid propane are commingled with the cracked oxidized bottoms at temperatures preferably above room temperature and under pressure sufficient to maintain the propane in a liquid state, the wax separation aids precipitate from solution while oil and wax constituents are dissolved by the propane. By allowing the mixture to remain in a quiescent state in a settling chamber, these wax separation aids settle to the bottom of the settling chamber and may be separated from the solution of propane, oil and wax by simple decantation of the solution. The propane, oil and wax solution may then be refrigerated in order to precipitate the wax which may then be separated by filtering, settling or centrifuging as previously described.

If desired, the wax separation aids may be precipitated along with the wax by chilling a solution of diluent such as propane and the cracked oxidized wax bottoms to a dewaxing temperature and then separating the precipitated mixture of precipitated wax and wax separation aids by filtration, cold settling or centrifuging. The precipitate may then be mixed with a solvent at a higher temperature in order to dissolve the wax from the mixture but to leave the wax separation aids as an undissolved fraction. By allowing

the mixture to remain in a quiescent state in a container, the undissolved wax separation aids will settle to the bottom of the container thereby permitting the solution of solvent and wax to be decanted from the settled wax separation aids. As solvents for this purpose, I may use liquid propane or any of the solvents heretofore mentioned at a temperature sufficient to accomplish the desired separation. If desired, the separation may be accomplished by means of a selective solvent capable of dissolving the wax separation aids but not appreciable amounts of wax, in which case, the mixture of wax, wax separation aids and solvent is permitted to stratify in two distinct layers, i. e. a layer of wax containing a small amount of the selective solvent and a layer of solvent in which the wax separation aids are dissolved. By separating the two layers, the wax separation aids may be recovered by distilling off the solvent from the layer containing them. As solvents for this purpose, I may use phenol, liquid sulfur dioxide, furfural or any of the solvents now known for separating oil into paraffinic and non-paraffinic oils.

I have also discovered that the cracked oxidized wax, in particular, the bottoms resulting from the cracking distillation of the oxidized wax, may be converted into effective wax modifiers, or wax separation aids by a condensation treatment of the cracked fraction alone or in the presence of aromatic hydrocarbons such as naphthalene, benzol and the like, through the influence of a polymerization catalyst such as aluminum chloride. Such a condensation treatment is well known in the condensation of chlorinated waxes. The condensation may be effected by mixing the cracked oxidized wax with about 20% by weight of naphthalene, for example, and 25% of aluminum chloride on the basis of the bottoms treated, and adding a sufficient amount of cleaners' naphtha or kerosene at 130° F. to 140° F. to completely dissolve the cracked oxidized wax and naphthalene. The reaction is allowed to continue for about 4 to 5 hours at which time the aluminous sludge is allowed to settle and the liquid fraction is withdrawn and distilled to remove the cleaners' naphtha or kerosene from the liquid fraction which comprises the wax modifier or wax separation aid. I have also discovered that the cracked oxidized bottoms when subjected to the aforementioned treatment with aluminum chloride may be made to yield a high percentage of lubricating oil of high viscosity index. This oil will have a higher viscosity than oil produced from the cracked bottoms without having been subjected to this treatment.

Instead of subjecting the entire cracked oxidized wax bottoms to the condensation treatment, I have found that an effective wax modifier may be produced by merely subjecting the wax separation aids free from oil and wax heretofore described, to the condensation treatment with aluminum chloride with or without the presence of the aromatic hydrocarbon. Thus, the cracked oxidized bottoms may be mixed with a solvent adapted to precipitate the wax separation aid and to dissolve the oil and wax components, as previously described, and the solution removed from the precipitated wax separation aids. These may then be subjected to the condensation treatment in the presence of aluminum chloride and with or without the aromatic hydrocarbon.

The cracking of the oxidized wax may be controlled so as to produce a sufficient amount of wax modifiers and lubricating oil of high vis-

cosity index. The cracked product after being freed of light oil fractions may then be blended with waxy lubricating oil to be dewaxed in a sufficient amount to provide the necessary amount of wax modifier. The mixture is then dewaxed. In this manner, the lubricating oil contained in the cracked products will be recovered along with the dewaxed oil and thus, in general, the viscosity index of the lubricating oil which was subjected to the dewaxing process will be increased due to the presence of the lubricating oil recovered from the cracked material.

From the foregoing, it will be seen that it is an object of my invention to oxidize paraffin wax and to subject the oxidized wax to a cracking or pyrogenic treatment for the purpose of recovering a lubricating oil of high viscosity index.

It is a further object of my invention to recover a wax modifier or wax separation aid from cracked oxidized paraffin wax.

Another object of my invention resides in cracking petroleum waxes which have been carefully and sufficiently oxidized at comparatively low temperatures, with or without the use of catalysts and with limited contact with air or oxygen and then recovering a high viscosity index lubricating oil and/or a wax separation aid from the cracked material.

A further object of my invention resides in subjecting oxidized waxes to a cracking treatment followed by a condensation treatment with aluminum chloride with or without the presence of an aromatic hydrocarbon.

Many specific objects, features and advantages of my invention will become apparent to those skilled in the art as the description of the invention proceeds in connection with specific examples given below which are not considered as limiting my invention but merely illustrative of methods of carrying it out.

#### Example 1

A charge of scale wax having a melting point of 123° F. was heated in a still to a temperature of 250° F. in the presence of 0.5% by weight of nickel naphthenate. Air was then introduced into the charge at a rate of 10 liters per hour for each 500 ml. of the wax and was continued for a period of 360 hours while maintaining the above temperature. The oxidized wax upon completion of the run showed an A. P. I. gravity of 23.9°, a saponification number of 157 and an acid number of 41.

Upon completion of the oxidation run, the charge was placed in a cracking still and heated to about 532° F. This temperature was gradually increased to about 630° F. During this heating period only the lighter unoxidized portion of the wax and the light oil fractions formed by the oxidation reaction were distilled. No reflux condensation was provided during this period. These fractions were recovered separately from the subsequent cracking and distillation treatment. The distillation was continued without a reflux condenser for about another hour at a temperature of 640-690° F. after which an air reflux condenser was provided and the cracking and distillation was continued for another three hours. During the last four hours of cracking and distillation, approximately 7.10% of oil and 2.03% of water were collected as condensate. The cracking and distillation was continued for another hour without a reflux condenser at a temperature of 690-712° F. and 3.04% of oil was collected as condensate. The 7.10% and 3.04%

5 of recovered oils were combined and showed an A. P. I. gravity of 44.6° at 60° F. The remaining bottoms comprised about 36.0% of the charge of oxidized wax. A portion of these bottoms were 10 mixed with 4 1/3 volumes of propane at 150° F. under a pressure of 330 pounds per square inch and the mixture was chilled by indirect heat exchange with solid CO<sub>2</sub> in a kerosene bath to about -40° F. This mixture was then filtered. The filtrate 15 was stripped of propane. Approximately 37.5% of dewaxed oil was recovered having an A. P. I. gravity of 28.5 at 60° F., a pour point of about 10° F., a viscosity of 148.4 seconds Saybolt Universal at 100° F. and 45.2 seconds at 210° F. indicating a viscosity index of about 133.0 and a viscosity gravity constant of 0.825.

#### Example 2

1% by weight of the material left in the filter 20 in Example 1, comprising a mixture of wax and wax modifier, was mixed at 300° F. with a waxy vacuum distilled lubricating oil from Santa Fe Springs crude oil, which had been refined by a treatment with phenol. The resulting mixture was then mixed with approximately 3 volumes of 25 liquid propane under superatmospheric pressure. The temperature of the resulting mixture was about 150° F. and the pressure was about 330 lbs. per square inch. The mixture of waxy lubricating oil, propane and added material was 30 then chilled externally at a rate of approximately 3° F. per minute to approximately -40° F., the refrigeration being accomplished by indirect heat exchange with solid CO<sub>2</sub> in a kerosene bath. The 35 chilled slurry of propane, lubricating oil, solidified wax and added material was filtered under a pressure of about 30 to 40 lbs. per square inch to effect the separation of the precipitated wax and added material from the propane solution of lubricating oil. The filter rate was 9 gallons per 40 square foot of filter surface per hour based on the propane free oil. It will be observed that all determinations of filter rates discussed herein are based on the dewaxed oil after separating the 45 propane therefrom. The filtrate was then distilled to remove the propane. Approximately 67% by volume of dewaxed oil was recovered having a pour point of 5° F. The separated wax had a melting point of 140° F.

50 In a dewaxing run under similar conditions but without any dewaxing aid the yield of dewaxed oil was 41% by volume and the filter rate 19.5 gallons/sq. ft./hr. The pour point of the oil was 5° F. and the melting point of the wax was 55 136° F.

#### Example 3

1% of the cracked oxidized bottoms produced 60 in Example 1, prior to the separation of oil therefrom, were mixed with another portion of the phenol raffinate described in Example 2 and the mixture was dewaxed in accordance with the procedure outlined in Example 2. Approximately 69.8% by volume of dewaxed oil was obtained having a pour point of 5° F. The filter rate was about 12.3 gallons per square foot per hour. The separated wax had a melting point of approximately 142° F.

#### Example 4

Another portion of the cracked oxidized wax bottoms produced in Example 1 were mixed with 20% by weight of naphthalene and with 4 1/2 volumes of cleaners' naphtha. Approximately 25% by weight of aluminum chloride, based on 75 the cracked bottoms, were added and the mixture

was maintained for 3 hours at 130° F. to 140° F. After the removal of the aluminous sludge and the cleaners' naphtha, the condensation product was considerably harder than the original oxidized wax bottoms.

Approximately 1% by weight of this was used to dewax the S. A. E. 40 phenol raffinate in accordance with the procedure of Example 2. Approximately 67.7% by volume of dewaxed oil was obtained having a pour point of 5° F. The filter rate was approximately 29.5 gallons per square foot per hour. The separated wax had a melting point of 142° F.

*Example 5*

Another portion of the cracked oxidized wax bottoms produced in Example 1 was subjected to a condensation treatment with aluminum chloride in accordance with the procedure of Example 4 except that the aromatic hydrocarbon, naphthalene, was omitted. The condensation product was somewhat less hard than that condensed with the aromatic hydrocarbon.

Approximately 1% by weight of this wax modifier was used to dewax the S. A. E. 40 phenol raffinate in accordance with the procedure of Example 2. Approximately 68.3% by volume of dewaxed oil was obtained having a pour point of 0° F. The filter rate was approximately 9.7 gallons per square foot per hour. The separated wax had a melting point of 142° F.

*Example 6*

A charge of scale wax having a melting point of 125° F. was heated in an aluminum column to a temperature of 325° F. which was maintained for the period of the oxidation. Air was introduced into the charge at a rate of 10 cubic feet per minute per barrel of the charge for a period of 10 hours. The oxidized wax upon completion of the run showed an A. P. I. gravity of 26.4°, a saponification number of 96.8 and an acid number of 43.8.

The oxidized charge was then placed in a cracking still which was provided with a reflux condenser and was subjected to cracking for a period of about 13 hours, the temperature being gradually increased from about 500° F. to 700° F. during the period of cracking. During the cracking period about 10.3% of light oil fractions having an A. P. I. gravity of 43.3° and about 4.8% of water based on the oxidized wax were distilled from the charge undergoing oxidation. Upon completion of the cracking reaction, the reflux condenser was removed and the cracked oxidized charge was topped at 540° F. to 685° F. Approximately 17.1% based on the oxidized wax of light oil fractions having an A. P. I. gravity of 39.8° were separated from the cracked bottoms.

The remaining bottoms had an A. P. I. gravity of 28.7. These were separated into two portions. One portion was mixed with about 7 volumes of propane at 125° F. under pressure sufficient to maintain the propane in a liquid state and the mixture was allowed to settle. The soluble portion of the cracked bottoms was decanted from the precipitated resins and was stripped of propane. Approximately 86.8% of the treated portion was recovered as oil having an A. P. I. gravity of 30.6°. The propane soluble portion was then dewaxed in propane in accordance with the dewaxing procedure described in Example 1. Approximately 40.5% based on the bottoms was recovered as a lubricating oil having an A. P. I. gravity of 25.5°, a viscosity of 367.3 seconds Say-

bolt Universal at 100° F. and 60.7 seconds at 210° F., a Viscosity index of 119.1 and a viscosity gravity constant of .836. This oil fraction corresponds with an S. A. E. 30 lubricating oil.

5 The other half of the cracked bottoms wax polymerized with aluminum chloride as in Example 4 and were subsequently dersined in liquid propane to produce approximately 83.9% of oil based on the bottoms treated having an A. P. I. 10 gravity of 29.5°. This oil was then dewaxed as previously described to produce about 41.7% of an oil having an A. P. I. gravity of 25.5°, a viscosity of 577 seconds at 100° F. and 73.7 seconds at 210° F., a viscosity index of 114.3 and a viscosity 15 gravity constant of .83. This oil fraction corresponds with an S. A. E. 40 lubricating oil.

It will be observed that the foregoing description of my invention is not to be considered as limiting as many variations thereof may be made by those skilled in the art within the scope of the 20 following claims.

I claim:

1. A process for treating wax which comprises subjecting said wax to oxidation with an oxidizing agent to produce an oxidized wax, heating 25 said oxidized wax to a cracking temperature to crack said oxidized wax, commingling said cracked oxidized wax with a diluent to precipitate resinous material from said mixture, separating a solution of oil, wax and diluent from said precipitated resinous material, chilling said solution to precipitate wax, separating a solution of oil and diluent from said precipitated wax and separating diluent from said solution.

35 2. A process for treating scale wax which comprises subjecting said wax to oxidation with an oxidizing agent to produce an oxidized wax and subsequently heating said oxidized wax to a cracking temperature and cracking said oxidized 40 wax in substantially the liquid phase at said cracking temperature to produce undistilled bottoms containing a lubricating oil fraction of high viscosity index and recovering a lubricating oil fraction of high viscosity index by extraction 45 from the undistilled bottoms produced in the cracking step.

3. A process for treating scale wax which comprises subjecting said wax to oxidation with an oxidizing agent to produce an oxidized wax, heating 50 said oxidized wax to a cracking temperature and cracking said oxidized wax in substantially the liquid phase at said cracking temperature to produce undistilled bottoms containing a lubricating oil fraction of high viscosity index 55 and subjecting such undistilled bottoms to treatment including extraction of a lubricating oil fraction of high viscosity index and condensation with an aromatic hydrocarbon in the presence of a polymerization catalyst.

60 4. A process for treating scale wax which comprises subjecting said wax to oxidation with an oxidizing agent to produce an oxidized wax, heating said oxidized wax to a cracking temperature and cracking said oxidized wax in substantially 65 the liquid phase at said cracking temperature to produce undistilled bottoms containing a lubricating oil fraction of high viscosity index and subjecting undistilled bottoms from said cracked oxidized wax to condensation with an aromatic hydrocarbon in the presence of aluminum chloride and recovering a lubricating fraction of high viscosity index by extraction from the condensed undistilled bottoms from the cracking step.

70 5. A process for treating wax which comprises

subjecting said wax to oxidation with an oxidizing agent to produce an oxidized wax, heating said oxidized wax to a cracking temperature and cracking said oxidized wax in substantially the liquid phase at said cracking temperature to produce undistilled bottoms containing a lubricating oil fraction of high viscosity index and

subjecting undistilled bottoms from said cracked oxidized wax to condensation in the presence of a polymerization catalyst and recovering a lubricating fraction of high viscosity index by extraction from the condensed undistilled bottoms from the cracking step.

RALPH C. POLLOCK.